



US006008184A

# United States Patent [19]

Pluyter et al.

[11] Patent Number: **6,008,184**[45] Date of Patent: **Dec. 28, 1999**

[54] **BLOCK COPOLYMERS FOR IMPROVED VISCOSITY STABILITY IN CONCENTRATED FABRIC SOFTENERS**

[75] Inventors: **Johan Gerwin Lodewijk Pluyter**,  
Eureka, Calif.; **Myriam Gerarda Eeckhout**, Gent, Belgium

[73] Assignee: **The Procter & Gamble Company**,  
Cincinnati, Ohio

[21] Appl. No.: **08/809,683**

[22] PCT Filed: **Sep. 1, 1995**

[86] PCT No.: **PCT/US95/11172**

§ 371 Date: **Apr. 28, 1998**

§ 102(e) Date: **Apr. 28, 1998**

[87] PCT Pub. No.: **WO96/10671**

PCT Pub. Date: **Apr. 11, 1996**

## [30] Foreign Application Priority Data

Sep. 30, 1994 [EP] European Pat. Off. .... 94870155

[51] Int. Cl.<sup>6</sup> ..... **D06M 15/00**; D06M 15/19

[52] U.S. Cl. ..... **510/524**; 510/461; 510/475;  
510/515; 510/522

[58] Field of Search ..... 510/515, 461,  
510/475, 522, 524

## [56] References Cited

### U.S. PATENT DOCUMENTS

|           |         |                  |       |         |
|-----------|---------|------------------|-------|---------|
| 4,429,859 | 2/1984  | Steiner et al.   | ..... | 510/524 |
| 4,702,857 | 10/1987 | Gosselink        | ..... | 510/299 |
| 4,767,547 | 8/1988  | Straathof et al. | ..... | 510/517 |
| 5,281,355 | 1/1994  | Tsaur et al.     | ..... | 510/393 |
| 5,510,042 | 4/1996  | Hartman et al.   | ..... | 510/516 |
| 5,767,062 | 6/1998  | Trinh et al.     | ..... | 510/516 |

### FOREIGN PATENT DOCUMENTS

|              |         |                    |       |           |
|--------------|---------|--------------------|-------|-----------|
| 185 427      | 6/1986  | European Pat. Off. | ..    |           |
| 0 239 910 A2 | 10/1987 | European Pat. Off. | ..... | C11D 1/62 |
| 458599       | 11/1991 | European Pat. Off. | ..    |           |

Primary Examiner—Anthony Green  
Attorney, Agent, or Firm—Robert B. Aylor

## [57] ABSTRACT

Liquid fabric softener compositions containing a combination of certain block copolymers and water soluble polymers to provide excellent storage stability and viscosity characteristics, especially at elevated temperatures.

**8 Claims, No Drawings**

**BLOCK COPOLYMERS FOR IMPROVED  
VISCOSITY STABILITY IN CONCENTRATED  
FABRIC SOFTENERS**

**TECHNICAL FIELD**

The present invention relates to fabric softener compositions to be used during the rinse cycle of a textile laundering operation to provide fabric softening/static control benefits.

The fabric softening compositions comprise beyond the conventional softener ingredients one or more polymers having a hydrophobic backbone with one or more hydrophilic side chains and are characterized by excellent storage stability and viscosity characteristics.

**BACKGROUND OF THE INVENTION**

Fabric softener compositions, especially concentrated and/or superconcentrated, are dispersions of positively charged vesicles containing the softener active. These vesicles are believed to be comprised of alternating concentric layers of water and lamellar cationic bilayers, so-called lamellar droplets. The presence of lamellar droplets in a fabric-softening composition can be detected by methods known to persons skilled in the art like optical techniques, rheometrical measurements, X-ray diffraction and electron microscopy. The droplets consist of an onion-like configuration of, as pointed out above, concentric bilayers of molecules of fabric-softening material with entrapped water or electrolyte solution, the so-called aqueous phase.

A well-appreciated fabric softener product exists of physical stability and desirable flow properties combined in one system.

However, upon storage the dispersions above-mentioned are thickening and eventually gelling. The reason for this phenomenon is not yet clear. There are, at least, two theoretical possibilities: the lamellar vesicles are increasingly interconnecting with time and eventually (1) form an infinitely inter-connected vesicle network or gel, or (2) change from a lamellar vesicle to a two-phase lamellar phase in which gelation may occur.

Regardless of the mechanism, gelation probably will be avoided as long as the vesicles are kept separated from each other.

It is well-known that two factors mainly determine the viscosity and stability of the fabric softening composition. First of all, it is the volume (fraction) of the dispersed lamellar phase in the composition and secondly it depends on the state of aggregation of these droplets. In general, the higher the volume (fraction) of the droplets (dispersed lamellar phase), the higher the viscosity which, if too high, results in an unpourable product. One way to solve this problem is using electrolytes whereby apparently the size of the lamellar vesicles is reduced and, as such, increases the inter-vesicle distances preventing aggregation/gelation.

However, the stability of other components in the fabric-softener composition is affected using higher electrolyte levels.

So there are limits to the amount of fabric softening material and electrolyte to be used whilst still having an acceptable product. There is a continued need for more concentrated, sometimes superconcentrated, fabric softening compositions for convenience and cost reduction purposes. The problem to be solved is that these high concentrations of softener active in the compositions must have an acceptable stability and at the same time pourability upon use.

**SUMMARY OF THE INVENTION**

We have now found that, with respect to the stability and viscosity requirements especially at elevated temperature, a fabric softening composition having conventional softener ingredients can be surprisingly favourable influenced by incorporating a block copolymer comprising a hydrophobic backbone with one or more hydrophilic side chains in the presence of a non-ionic water soluble polymer. These polymeric materials reduce the viscosity of concentrated dispersions of cationic softener actives in lamellar vesicles and improves unexpected the stabilizing properties of the fabric softening compositions. As such, they prevent these types of formulations from gelling or solidifying. Another practical benefit of these materials is that they prevent skin formation and dispenser residue upon use.

Furthermore, we have found that the use of a block copolymer with a hydrophobic backbone and one or more hydrophilic side chains according to the invention in a fabric softener composition, reduces the viscosity of the composition at low and high temperature as well.

**DETAILED DESCRIPTION OF THE  
INVENTION**

The objective of polymer stabilization in concentrated fabric softener formulations is to maintain low viscosity upon storage at low (0° C.) and high (50° C.) temperatures without affecting the softening performance. It appears that so-called di- and tri-block copolymers of the types A-B and A-B-A, respectively, and preferably tri-block copolymers with highly water-soluble blocks (A) and an insoluble or partially water-soluble blocks (B) in combination with a very water-soluble polymer (cloud point larger than 90° C.) provides excellent viscosity stabilization of concentrated compositions. The block copolymers are defined as: (a) separated polymer blocks (of more than two units) of the same kind separated by, at least, one monomer of another kind, (b) different kinds of polymer blocks of more than two monomers that are chemically connected. Probably a mixed depletion/steric stabilization phenomenon is likely to be responsible for this behavior. Key parameters in the structure of these materials are (1) the chain lengths of the blocks, (2) the water-solubility of the blocks, and (3) the specific interactions of the B blocks with the lamellar vesicles. In addition, we have also found that said di- or tri-block copolymers without the water-soluble polymer provide excellent viscosity stabilization especially at high elevated temperature.

The following five general polymer structures (I-V) provide above-mentioned viscosity stabilization:

- (I) polymers that are likely to adhere physically to the positively charged vesicle surface: C-(A)<sub>x</sub>-(B)<sub>y</sub>-D and C-(A)<sub>x</sub>-(B)<sub>y</sub>-(A)<sub>z</sub>-D, where the monomers A and B are water soluble and partially water insoluble respectively, and C and D are end groups or a hydrogen atom. Typical end groups are hydroxyl, acetate, methyl amine or quaternary amine.
- (II) Polymers that are likely to be incorporated into the lamellar vesicles: D-(A)<sub>x</sub>-R-(A)<sub>z</sub>-C, where R is a polymer of B monomers as defined above, or preferably a fatty alcohol or acid of which one carbon atom is substituted with polymer blocks. For instance, the mono fatty ester of ethoxylated glycerol.
- (III) Combinations of polymers of type (I) and (II) with nonionic water soluble polymers, such as polyvinyl pyrrolidone, polyvinyl pyridine-N-oxide, polyethylene glycol, and substituted poly alcohol.

Further details about these polymer structures are described below.

(IV) Polymer combinations amongst type (I), amongst type (II) and mixed type (I)+type (II) combinations.

(V) Combinations of (III) and (IV).

In EP 458 599, an attempt is made to solve the problem of stability and acceptable viscosity of the finished product. A fabric treatment composition is disclosed therein comprising an aqueous base, one or more, fabric-softening materials and an emulsion component. The composition has a structure of lamellar droplets of the fabric-softening material in combination with an emulsion, said composition also comprises a deflocculating polymer of a hydrophilic backbone and one or more hydrophobic sidechains.

However, it appears that using these types of polymers (block copolymers), the presumed right system for ideal steric stabilization is not created. This steric stabilization mechanism requires that the polymer chains, which are soluble in the continuous phase, are physically or chemically grafted onto the particle surface. The remaining part of the polymer (the stabilizing polymer chain) is, ideally, pointing away from the particle surface. In a sterically stabilized dispersion of particles, these stabilizing polymer chains are rejecting each others presence in the continuous phase. The following mechanism is generally accepted for steric stabilization. When the polymer-water (continuous phase) and water-water molecular interactions are much higher than the polymer-polymer interactions (water solubility requirements) there occurs some kind of microphase separation. Of course, there are not two separate phases present, but at the molecular level the polymer molecules remain separated. If, on the other hand, polymer-polymer interactions are larger than polymer-water interactions, the polymer chains of different particles will attract each other, and will cause destabilization of the dispersion. The phenomenon appears as a repulsive interaction between the polymer chains (steric stabilization).

Key parameters for this type of stabilization are:

- (a) the stabilizing polymer chains must be very soluble in the continuous phase, while the attached part of the polymer must be insoluble;
- (b) the stabilizing polymer chain must be of a minimum (and optimum) length in order to stabilize the dispersion efficiently.

Both conditions are not met by applying the polymers as described in EP 458, 599.

We have found that block copolymers with cloud points ranging from 40° C. and higher are able to stabilize aqueous dispersions of lamellar vesicles. The cloud point dependence is caused by the chain length of the water-soluble and insoluble blocks, as well as the ratio of the two chain lengths. The insoluble blocks may be as hydrophobic as poly propylene oxide (PO) ranging from aliphatic/aromatic polyesters to aliphatic chains. When the chain lengths are too short, e.g. (A)x blocks with x<20 and (B)y blocks with y=3, the opposite of viscosity stabilization occurs; extreme thickening or even gelation takes place.

The level of these types of polymers ranges from 0.1–10%, preferably 0.1–5%, and even more preferable 0.5–2%.

In EP 0 185 427 (Gosselink) these polymers are described in the context of soil release polymer in fabric softening composition. We have found a new use of these polymers viz. the reduction of viscosity of the composition at low and elevated temperature. Surprisingly the compositions remain stable with respect to the viscosity as well.

In addition, these polymers prevent skin formation. This occurs through specific complexation of water molecules

with the water-soluble polymer blocks. This complexation with water reduces the vapour pressure of water, which slows down or even prevents skin formation. Examples of such cases are block copolymers with poly ethoxylate, polyvinyl pyrrolidone, and polyvinyl pyridine-N-oxide (ethoxylated and/or partially cationic) blocks. The best molecular weight range of the water-soluble blocks for minimum skin formation ranges from 100–20000, preferably from 2000–8000.

The polymers may be added at any point in the process. However, this is dependent on the formulation matrix. Three points of addition are preferred: (1) to the water seat, (2) on top of the formulation before or after the perfume addition (hot or cold), (3) a combination of (1) and (2). Preferred is the point of addition (1) which, probably assists the incorporation of the polymer in the vesicle structure. The best ways of addition are via the water seat or afterwards while hot (40–90° C.) or ambient.

#### Type I Polymers

The polymers of type I likely to adhere to the positively charged vesicle surface have the general formula (1) C-(A)x-(B)y-D and formula (2) C-(A)x-(B)y-(A)z-D respectively viz. so-called di- and triblock copolymers.

The monomers A and B are water soluble and partially water insoluble groups, respectively. The degrees of polymerization x and z are preferably of the same order of magnitude. The structural parameters x and z are from 1–200, preferably 30–60; y ranges from 1–70, preferably from 3–40. C and D are end groups and may be selected from the same series of groups. However, some situations require them to be different.

#### Possible Types of Monomers for A (Water-soluble as Polymers):

Ethylene oxide

Vinylpyrrolidone

Vinyl 2- and 4-pyridine

Vinyl 2- and 4-pyridine-N-oxide

Cationic 2- and 4-vinyl pyridine



40  
45  
50  
55  
518  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
670  
671  
672  
673  
674  
675  
676  
677  
678  
679  
680  
681  
682  
683  
684  
685  
686  
687  
688  
689  
690  
691  
692  
693  
694  
695  
696  
697  
698  
699  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
730  
731  
732  
733  
734  
735  
736  
737  
738  
739  
740  
741  
742  
743  
744  
745  
746  
747  
748  
749  
750  
751  
752  
753  
754  
755  
756  
757  
758  
759  
760  
761  
762  
763  
764  
765  
766  
767  
768  
769  
770  
771  
772  
773  
774  
775  
776  
777  
778  
779  
7710  
7711  
7712  
7713  
7714  
7715  
7716  
7717  
7718  
7719  
7720  
7721  
7722  
7723  
7724  
7725  
7726  
7727  
7728  
7729  
7730  
7731  
7732  
7733  
7734  
7735  
7736  
7737  
7738  
7739  
7740  
7741  
7742  
7743  
7744  
7745  
7746  
7747  
7748  
7749  
7750  
7751  
7752  
7753  
7754  
7755  
7756  
7757  
7758  
7759  
7760  
7761  
7762  
7763  
7764  
7765  
7766  
7767  
7768  
7769  
7770  
7771  
7772  
7773  
7774  
7775  
7776  
7777  
7778  
7779  
77710  
77711  
77712  
77713  
77714  
77715  
77716  
77717  
77718  
77719  
77720  
77721  
77722  
77723  
77724  
77725  
77726  
77727  
77728  
77729  
77730  
77731  
77732  
77733  
77734  
77735  
77736  
77737  
77738  
77739  
77740  
77741  
77742  
77743  
77744  
77745  
77746  
77747  
77748  
77749  
77750  
77751  
77752  
77753  
77754  
77755  
77756  
77757  
77758  
77759  
77760  
77761  
77762  
77763  
77764  
77765  
77766  
77767  
77768  
77769  
77770  
77771  
77772  
77773  
77774  
77775  
77776  
77777  
77778  
77779  
77780  
77781  
77782  
77783  
77784  
77785  
77786  
77787  
77788  
77789  
77790  
77791  
77792  
77793  
77794  
77795  
77796  
77797  
77798  
77799  
777100  
777101  
777102  
777103  
777104  
777105  
777106  
777107  
777108  
777109  
777110  
777111  
777112  
777113  
777114  
777115  
777116  
777117  
777118  
777119  
777120  
777121  
777122  
777123  
777124  
777125  
777126  
777127  
777128  
777129  
777130  
777131  
777132  
777133  
777134  
777135  
777136  
777137  
777138  
777139  
777140  
777141  
777142  
777143  
777144  
777145  
777146  
777147  
777148  
777149  
777150  
777151  
777152  
777153  
777154  
777155  
777156  
777157  
777158  
777159  
777160  
777161  
777162  
777163  
777164  
777165  
777166  
777167  
777168  
777169  
777170  
777171  
777172  
777173  
777174  
777175  
777176  
777177  
777178  
777179  
777180  
777181  
777182  
777183  
777184  
777185  
777186  
777187  
777188  
777189  
777190  
777191  
777192  
777193  
777194  
777195  
777196  
777197  
777198  
777199  
777200  
777201  
777202  
777203  
777204  
777205  
777206  
777207  
777208  
777209  
777210  
777211  
777212  
777213  
777214  
777215  
777216  
777217  
777218  
777219  
777220  
777221  
777222  
777223  
777224  
777225  
777226  
777227  
777228  
777229  
777230  
777231  
777232  
777233  
777234  
777235  
777236  
777237  
777238  
777239  
777240  
777241  
777242  
777243  
777244  
777245  
777246  
777247  
777248  
777249  
777250  
777251  
777252  
777253  
777254  
777255  
777256  
777257  
777258  
777259  
777260  
777261  
777262  
777263  
777264  
777265  
777266  
777267  
777268  
777269  
777270  
777271  
777272  
777273  
777274  
777275  
777276  
777277  
777278  
777279  
777280  
777281  
777282  
777283  
777284  
777285  
777286  
777287  
777288  
777289  
777290  
777291  
777292  
777293  
777294  
777295  
777296  
777297  
777298  
777299  
777300  
777301  
777302  
777303  
777304  
777305  
777306  
777307  
777308  
777309  
777310  
777311  
777312  
777313  
777314  
777315  
777316  
777317  
777318  
777319  
777320  
777321  
777322  
777323  
777324  
777325  
777326  
777327  
777328  
777329  
777330  
777331  
777332  
777333  
777334  
777335  
777336  
777337  
777338  
777339  
777340  
777341  
777342  
777343  
777344  
777345  
777346  
777347  
777348  
777349  
777350  
777351  
777352  
777353  
777354  
777355  
777356  
777357  
777358  
777359  
777360  
777361  
777362  
777363  
777364  
777365  
777366  
777367  
777368  
777369  
777370  
777371  
777372  
777373  
777374  
777375  
777376  
777377  
777378  
777379  
777380  
777381  
777382  
777383  
777384  
777385  
777386  
777387  
777388  
777389  
777390  
777391  
777392  
777393  
777394  
777395  
777396  
777397  
777398  
777399  
777400  
777401  
777402  
777403  
777404  
777405  
777406  
777407  
777408  
777409  
777410  
777411  
777412  
777413  
777414  
777415  
777416  
777417  
777418  
777419  
777420  
777421  
777422  
777423  
777424  
777425  
777426  
777427  
777428  
777429  
777430  
777431  
777432  
777433  
777434  
777435  
777436  
777437  
777438  
777439  
777440  
777441  
777442  
777443  
777444  
777445  
777446  
777447  
777448  
777449  
777450  
777451  
777452  
777453  
777454  
777455  
777456  
777457  
777458  
777459  
777460  
777461  
777462  
777463  
777464  
777465  
777466  
777467  
777468  
777469  
777470  
777471  
777472  
777473  
777474  
777475  
777476  
777477  
777478  
777479  
777480  
777481  
777482  
777483  
777484  
777485  
777486  
777487  
777488  
777489  
777490  
777491  
777492  
777493  
777494  
777495  
777496  
777497  
777498  
777499  
777500  
777501  
777502  
777503  
777504  
777505  
777506  
777507  
777508  
777509  
777510  
777511  
777512  
777513  
777514  
777515  
777516  
777517  
777518  
777519  
777520  
777521  
777522  
777523  
777524  
777525  
777526  
777527  
777528  
777529  
777530  
777531  
777532  
777533  
777534  
777535  
777536  
777537  
777538  
777539  
777540  
777541  
777542  
777543  
777544  
777545  
777546  
777547  
777548  
777549  
777550  
777551  
777552  
777553  
777554  
777555  
777556  
777557  
777558  
777559  
777560  
777561  
777562  
777563  
777564  
777565  
777566  
777567  
777568  
777569  
777570  
777571  
777572  
777573  
777574  
777575  
777576  
777577  
777578  
777579  
777580  
777581  
777582  
777583  
777584  
777585  
777586  
777587  
777588  
777589  
777590  
777591  
777592  
777593  
777594  
777595  
777596  
777597  
777598  
777599  
777600  
777601  
777602  
777603  
777604  
777605  
777606  
777607  
777608  
777609  
777610  
777611  
777612  
777613  
777614  
777615  
777616  
777617  
777618  
777619  
777620  
777621  
777622  
777623  
777624  
777625  
777626  
777627  
777628  
777629  
777630  
777631  
777632  
777633  
777634  
777635  
777636  
777637  
777638  
777639  
777640  
777641  
777642  
777643  
777644  
777645  
777646  
777647  
777648  
777649  
777650  
777651  
777652  
777653  
777654  
777655  
777656  
777657  
777658  
777659  
777660  
777661  
777662  
777663  
777664  
777665  
777666  
777667  
777668  
777669  
777670  
777671  
777672  
777673  
777674  
777675  
777676  
777677  
777678  
777679  
777680  
777681  
777682  
777683  
777684  
777685  
777686  
777687  
777688  
777689  
777690  
777691  
777692  
777693  
777694  
777695  
777696  
777697  
777698  
777699  
777700  
777701  
777702  
777703  
777704  
777705  
777706  
777707  
777708  
777709  
777710  
777711  
777712  
777713  
777714  
777715  
777716  
777717  
777718  
777719  
777720  
777721  
777722  
777723  
777724  
777725  
777726  
777727  
777728  
777729  
777730  
777731  
777732  
777733  
777734  
777735  
777736  
777737  
777738  
777739  
777740  
777741  
777742  
777743  
777744  
777745  
777746  
777747  
777748  
777749  
777750  
777751  
777752  
777753  
777754  
777755  
777756  
777757  
777758  
777759  
777760  
777761  
777762  
777763  
777764  
777765  
777766  
777767  
777768  
777769  
777770  
777771  
777772  
777773  
777774  
777775  
777776  
777777  
777778  
777779  
777780  
777781  
777782  
777783  
777784  
777785  
777786  
777787  
777788  
777789  
777790  
777791  
777792  
777793  
777794  
777795  
777796  
777797  
777798  
777799  
777800  
777801  
777802  
777803  
777804  
777805  
777806  
777807  
777808  
777809  
777810  
777811  
777812  
777813  
777814  
777815  
777816  
777817  
777818  
777819  
777820  
777821  
777822  
777823  
777824  
777825  
777826  
777827  
777828  
777829  
777830  
777831  
777832  
777833  
777834  
777835  
777836  
777837  
777838  
777839  
777840  
777841  
777842  
777843  
777844  
777845  
777846  
777847  
777848  
777849  
777850  
777851  
777852  
777853  
777854  
777855  
777856  
777857  
777858  
777859  
777860  
777861  
777862  
777863  
777864  
777865  
777866  
777867  
777868  
777869  
777870  
777871  
777872  
777873  
777874  
777875  
777876  
777877  
777878  
777879  
777880  
777881  
777882  
777883  
777884  
777885  
777886  
777887  
777888  
777889  
777890  
777891  
777892  
777893  
777894  
777895  
777896  
777897  
777898  
777899  
777900  
777901  
777902  
777903  
777904  
777905  
777906  
777907  
777908  
777909  
777910  
777911  
777912  
777913  
777914  
777915  
777916  
777917  
777918  
777919  
777920  
777921  
777922  
777923  
777924  
777925  
777926  
777927  
777928  
777929  
777930  
777931  
777932  
777933  
777934  
777935  
777936  
777937  
777938  
777939  
777940  
777941  
777942  
777943  
777944  
777945  
777946  
777947  
777948  
777949  
777950  
777951  
777952  
777953  
777954  
777955  
777956  
777957  
777958  
777959  
777960  
777961  
777962  
777963  
777964  
777965  
777966  
777967  
777968  
777969  
777970  
777971  
77797

Poly(alkylene terephthalate) where the alkylene group may be C1–C10, preferably C2–C4.  
 Aliphatic polyesters, —O—(CH<sub>2</sub>)<sub>n</sub>—CO—, where n=1–10, preferably 1–4.  
 Polybutadiene  
 Hydroxylated polybutadiene  
 Straight saturated and unsaturated aliphatic chains, carbon chain length C4–50, preferably C4–20.  
 Poly (3-hydroxybutyric acid), degrees of polymerization of 4–50, preferably 4–30.  
 Aliphatic/aromatic or mixed carbonates  
 Esterified polysaccharides  
 Polysiloxanes  
 Polyurethanes  
 Polyacrylates  
 Cellulose derivatives, such as chitosans.  
 Possible end Groups C and D:  
 Hydrogen atoms  
 Hydroxyl groups  
 Alkoxy groups, —O—R—, where R=H, saturated or partially unsaturated aliphatic alkanes  
 Methyl groups  
 Alkyl groups  
 —CH(CH<sub>3</sub>)<sub>2</sub>, —CH<sub>2</sub>(CH<sub>3</sub>), —C(CH<sub>3</sub>)<sub>3</sub>  
 Alkyl chains straight chain saturated and unsaturated fatty alcohol/acid, chain length C4–50, preferably C4–20.  
 Cationic end groups, such as —CH<sub>2</sub>—CO—N<sup>+</sup>(CH<sub>3</sub>)<sub>3</sub> X—, where X is a halide ion, methyl, sulphate or acetate.  
 —O—CO—(CH<sub>2</sub>)<sub>n</sub>—CH<sub>3</sub>, where n=2–30, preferably 2–20.  
 Sulphonate groups.  
 Type II Polymers  
 These polymers are likely to be partially incorporated into the positively charged vesicle and have the following general structure of formula (3):



A, x, z, C, and D are defined as in type I polymers.

P is a glycerol or other polyalcohol unit such as poly(vinyl)alcohol or polysaccharides or the one shown below.



Other types of polymers that are likely to be partially incorporated in the lamellar vesicles when stabilizing dispersions are shown below (a substituted polyglycerol).



In these polymer types, R can be a polymer of the monomers of type B, but is preferred to be a saturated or unsaturated fatty acid, n=1–10, preferably 1–8, and m=1–10, preferably 1–5. The hydroxyl end groups may be replaced by the end groups C and D, as defined in the previous polymer types.

Improved viscosity stabilization at low and elevated temperature as well occurs by using mixtures of completely

water-soluble polymers and di- or tri-block copolymers according to the invention.

The viscosity stabilizing properties of di-and tri-block copolymers of the types I and II, or polymers mentioned in EP 0 185 427 (E. P. Gosselink), or mixtures thereof, can be improved by addition of small amounts of completely water-soluble polymers (cloud point larger than 90° C.), such as poly vinyl pyrrolidone, polyvinyl pyridine-N-oxide, polyethylene glycol, substituted poly glycerols. The weight % of di- or tri-block copolymers in the formulation ranges from 0.1–10%, preferably from 0.2–6%. The weight % of completely water-soluble non-ionic polymers in the formulation ranges from 0.1–10%, preferably from 0.2–6%.

Fabric conditioning compositions, in particular fabric softening compositions to be used in the rinse cycle of laundry washing processes, are well known.

The fabric softening materials may be selected from cationic, nonionic, amphoteric or anionic fabric softening material.

Compositions of the present invention preferably comprise from 1 to 80% by weight of fabric softening active, more preferably from 2 to 70% by weight, most preferably from 5 to 50% by weight of the composition.

Typically, such compositions contain a water-insoluble quaternary-ammonium fabric softening active, the most commonly used having been di-long alkyl chain ammonium chloride.

In recent years, the need has arisen for more environmentally-friendly materials, and rapidly biodegradable quaternary ammonium compounds have been presented as alternatives to the traditionally used di-long chain ammonium chlorides. Such quaternary ammonium compounds contain long chain alk(en)yl groups interrupted by functional groups such as carboxy groups.

Said materials and fabric softening compositions containing them are disclosed in numerous publications such as EPA 040 562, and EPA 239 910.

In EPA 239 910, it has been disclosed that a pH range of from 2.5 to 4.2 provides optimum storage stability to said rapidly biodegradable ammonium compounds.

The quaternary ammonium compounds and amine precursors herein have the formula (I) or (II), below:



Q is





$R^1$  is  $(\text{CH}_2)_n\text{---Q---T}^2$  or  $T^3$ ;  
 $R^2$  is  $(\text{CH}_2)_m\text{---Q---T}^4$  or  $T^5$  or  $R^3$ ;  
 $R^3$  is  $C_1\text{---C}_4$  alkyl or  $C_1\text{---C}_4$  hydroxyalkyl or H;  
 $R^4$  is H or  $C_1\text{---C}_4$  alkyl or  $C_1\text{---C}_4$  hydroxyalkyl;  
 $T_1, T^2, T^3, T^4, T^5$  are (the same or different)  $C_{11}\text{---C}_{22}$  alkyl or alkenyl;  
n and m are integers from 1 to 4; and  
 $X^-$  is a softener-compatible anion.

The alkyl, or alkenyl, chain  $T^1, T^2, T^3, T^4, T^5$  must contain at least 11 carbon atoms, preferably at least 16 carbon atoms. The chain may be straight or branched.

Tallow is a convenient and inexpensive source of long chain alkyl and alkenyl material. The compounds wherein  $T^1, T^2, T^3, T^4, T^5$  represents the mixture of long chain materials typical for tallow are particularly preferred.

Specific examples of quaternary ammonium compounds suitable for use in the aqueous fabric softening compositions herein include:

- 1)  $N,N$ -di(tallowoyl-oxy-ethyl)- $N,N$ -dimethyl ammonium chloride;
- 2)  $N,N$ -di(tallowoyl-oxy-ethyl)- $N$ -methyl,  $N$ -(2-hydroxyethyl);
- 3)  $N,N$ -di(2-tallowyloxy-2-oxo-ethyl)- $N,N$ -dimethyl ammonium chloride;
- 4)  $N,N$ -di(2-tallowyloxyethylcarbonyloxyethyl)- $N,N$ -dimethyl ammonium chloride;
- 5)  $N$ -(2-tallowyloxy-2-ethyl)- $N$ -(2-tallowyloxy-2-oxo-ethyl)- $N,N$ -dimethyl ammonium chloride;
- 6)  $N,N,N$ -tri(tallowyl-oxy-ethyl)- $N$ -methyl ammonium chloride;
- 7)  $N$ -(2-tallowyloxy-2-oxoethyl)- $N$ -(tallowyl- $N,N$ -dimethyl-ammonium chloride; and
- 8) 1,2-ditallowyl oxy-3-trimethylammoniopropane chloride.; and mixtures of any of the above materials.

Of these, compounds 1-7 are examples of compounds of Formula (I); compound 8 is a compound of Formula (II).

Particularly preferred is  $N,N$ -di(tallowoyl-oxy-ethyl)- $N,N$ -dimethyl ammonium chloride, where the tallow chains are at least partially unsaturated.

The level of unsaturation of the tallow chain can be measured by the Iodine Value (IV) of the corresponding fatty acid, which in the present case should preferably be in the range of from 5 to 100 with two categories of compounds being distinguished, having a IV below or above 25.

Indeed, for compounds of Formula (I) made from tallow fatty acids having a IV of from 5 to 25, preferably 15 to 20, it has been found that a cis/trans isomer weight ratio greater than about 30/70, preferably greater than about 50/50 and more preferably greater than about 70/30 provides optimal concentrability.

For compounds of Formula (I) made from tallow fatty acids having a IV of above 25, the ratio of cis to trans isomers has been found to be less critical unless very high concentrations are needed.

Other examples of suitable quaternary ammoniums of Formula (I) and (II) are obtained by, e.g.:

replacing "tallow" in the above compounds with, for example, coco, palm, lauryl, oleyl, ricinoleyl, stearyl, palmityl, or the like, said fatty acyl chains being either fully saturated, or preferably at least partly unsaturated; replacing "methyl" in the above compounds with ethyl, ethoxy, propyl, propoxy, isopropyl, butyl, isobutyl or t-butyl;

replacing "chloride" in the above compounds with bromide, methylsulfate, formate, sulfate, nitrate, and the like.

In fact, the anion is merely present as a counterion of the positively charged quaternary ammonium compounds. The nature of the counterion is not critical at all to the practice of the present invention. The scope of this invention is not considered limited to any particular anion.

By "amine precursors thereof" is meant the secondary or tertiary amines corresponding to the above quaternary ammonium compounds, said amines being substantially protonated in the present compositions due to the claimed pH values.

The quaternary ammonium or amine precursors compounds herein are present at levels of from about 1% to about 80% of compositions herein, depending on the composition execution which can be dilute with a preferred level of active from about 5% to about 15%, or concentrated, with a preferred level of active from about 15% to about 50%, most preferably about 15% to about 35%.

#### Optional Ingredients

25 Fully formulated fabric softening compositions preferably contain, in addition to the compounds of Formula I or II herein, one or more of the following ingredients:

30 Firstly, the presence of polymer having a partial or net cationic charge, can be useful to further increase the cellulase stability in the compositions herein. Such polymers can be used at levels of from 0.001% to 10%, preferably 0.01% to 2% by weight of the compositions.

35 Such polymers having a partial cationic charge can be polyamine N-oxide containing polymers which contain units having the following structure formula (A):



(A)

wherein P is a polymerisable unit, whereto the R—N—O group can be attached to or wherein the R—N—O group forms part of the polymerisable unit or a combination of both.

A is



x is 0 or 1;

60 R are aliphatic, ethoxylated aliphatics, aromatic, heterocyclic or alicyclic groups or any combination thereof whereto the nitrogen of the N—O group can be attached or wherein the nitrogen of the N—O group is part of these groups.

The N—O group can be represented by the following general structures:



wherein R<sup>1</sup>, R<sup>2</sup>, and R<sup>3</sup> are aliphatic groups, aromatic, heterocyclic or alicyclic groups or combinations thereof, x or/and y or/and z is 0 or 1 and wherein the nitrogen of the N→O group can be attached or wherein the nitrogen of the N→O group forms part of these groups.

The N→O group can be part of the polymerisable unit (P) or can be attached to the polymeric backbone or a combination of both.

Suitable polyamine N-oxides wherein the N→O group forms part of the polymerisable unit comprise polyamine N-oxides wherein R is selected from aliphatic, aromatic, alicyclic or heterocyclic groups.

One class of said polyamine N-oxides comprises the group of polyamine N-oxides wherein the nitrogen of the N→O group forms part of the R-group. Preferred polyamine N-oxides are those wherein R is a heterocyclic group such as pyridine, pyrrole, imidazole, pyrrolidine, piperidine, quinoline, acridine and derivatives thereof.

Another class of said polyamine N-oxides comprises the group of polyamine N-oxides wherein the nitrogen of the N→O group is attached to the R-group.

Other suitable polyamine N-oxides are the polyamine oxides whereto the N→O group is attached to the polymerisable unit.

Preferred class of these polyamine N-oxides are the polyamine N-oxides having the general formula (A) wherein R is an aromatic, heterocyclic or alicyclic groups wherein the nitrogen of the N→O functional group is part of said R group.

Examples of these classes are polyamine oxides wherein R is a heterocyclic compound such as pyridine, pyrrole, imidazole and derivatives thereof.

Another preferred class of polyamine N-oxides are the polyamine oxides having the general formula (A) wherein R are aromatic, heterocyclic or alicyclic groups wherein the nitrogen of the N→O functional group is attached to said R groups.

Examples of these classes are polyamine oxides wherein R groups can be aromatic such as phenyl.

Any polymer backbone can be used as long as the amine oxide polymer formed is water-soluble and has dye transfer inhibiting properties. Examples of suitable polymeric backbones are polyvinyls, polyalkylenes, polyesters, polyethers, polyamide, polyimides, polyacrylates and mixtures thereof.

The amine N-oxide polymers useful herein typically have a ratio of amine to the amine N-oxide of about 10:1 to about 1:1000000. However the amount of amine oxide groups present in the polyamine N-oxide containing polymer can be varied by appropriate copolymerization or by appropriate degree of N-oxidation. Preferably, the ratio of amine to amine N-oxide is from about 2:3 to about 1:1000000. More preferably from about 1:4 to about 1:1000000, most preferably from about 1:7 to about 1:1000000. The polymers of the present invention actually encompass random or block copolymers where one monomer type is an amine N-oxide and the other monomer type is either an amine N-oxide or not. The amine oxide unit of the polyamine N-oxides has a PKa<10, preferably PKa<7, more preferred PKa<6.

The polyamine N-oxide containing polymer can be obtained in almost any degree of polymerisation. The degree of polymerisation is not critical provided the material has the desired water-solubility and dye-suspending power.

Typically, the average molecular weight of the polyamine N-oxide containing polymer is within the range of about 500 to about 1000,000; preferably from about 1,000 to about 50,000, more preferably from about 2,000 to about 30,000, 5 most preferably from about 3,000 to about 20,000.

Such polymers having a net cationic charge include polyvinylpyrrolidone (PVP) as well as copolymers of N-vinylimidazole N-vinyl pyrrolidone, having an average molecular weight range in the range about 5,000 to about 10 100,000, preferably about 5,000 to about 50,000; said copolymers having a molar ratio of N-vinylimidazole to N-vinylpyrrolidone from about 1 to about 0.2, preferably from about 0.8 to about 0.3.

#### Other Optional Ingredients Include:

15 Additional Softening Agents: which are nonionic fabric softener materials. Typically, such nonionic fabric softener materials have a HLB of from about 2 to about 9, more typically from about 3 to about 7. Such nonionic fabric softener materials tend to be readily dispersed either by 20 themselves, or when combined with other materials such as single-long-chain alkyl cationic surfactant described in detail hereinafter. Dispersibility can be improved by using more single-long-chain alkyl cationic surfactant, mixture with other materials as set forth hereinafter, use of hotter 25 water, and/or more agitation. In general, the materials selected should be relatively crystalline, higher melting, (e.g.>40° C.) and relatively water-insoluble.

The level of optional nonionic softener in the compositions herein is typically from about 0.1% to about 10%, 30 preferably from about 1% to about 5%.

Preferred nonionic softeners are fatty acid partial esters of polyhydric alcohols, or anhydrides thereof, wherein the alcohol, or anhydride, contains from 2 to 18, preferably from 2 to 8, carbon atoms, and each fatty acid moiety contains 35 from 12 to 30, preferably from 16 to 20, carbon atoms. Typically, such softeners contain from one to 3, preferably 2 fatty acid groups per molecule.

The polyhydric alcohol portion of the ester can be ethylene glycol, glycerol, poly (e.g., di-, tri-, tetra-, penta-, and/or 40 hexa-) glycerol, xylitol, sucrose, erythritol, pentaerythritol, sorbitol or sorbitan. Sorbitan esters and polyglycerol monostearate are particularly preferred.

The fatty acid portion of the ester is normally derived from fatty acids having from 12 to 30, preferably from 16 to 20, carbon atoms, typical examples of said fatty acids being 45 lauric acid, myristic acid, palmitic acid, stearic acid and behenic acid.

Highly preferred optional nonionic softening agents for use in the present invention are the sorbitan esters, which are 50 esterified dehydration products of sorbitol, and the glycerol esters.

Commercial sorbitan monostearate is a suitable material. Mixtures of sorbitan stearate and sorbitan palmitate having 55 stearate/palmitate weight ratios varying between about 10:1 and about 1:10, and 1,5-sorbitan esters are also useful.

Glycerol and polyglycerol esters, especially glycerol, diglycerol, triglycerol, and polyglycerol mono- and/or di-esters, preferably mono-, are preferred herein (e.g. polyglycerol monostearate with a trade name of Radiasurf 7248).

60 Useful glycerol and polyglycerol esters include mono-esters with stearic, oleic, palmitic, lauric, isostearic, myristic, and/or behenic acids and the diesters of stearic, oleic, palmitic, lauric, isostearic, behenic, and/or myristic acids. It is understood that the typical mono-ester contains some di- and tri-ester, etc.

The "glycerol esters" also include the polyglycerol, e.g., diglycerol through octaglycerol esters. The polyglycerol

polyols are formed by condensing glycerin or epichlorohydrin together to link the glycerol moieties via ether linkages. The mono- and/or diesters of the polyglycerol polyols are preferred, the fatty acyl groups typically being those described hereinbefore for the sorbitan and glycerol esters.

#### Surfactant/Concentration Aids

Although as stated before, relatively concentrated compositions of the unsaturated material of Formula (I) and (II) above can be prepared that are stable without the addition of concentration aids, the concentrated compositions of the present invention may require organic and/or inorganic concentration aids to go to even higher concentrations and/or to meet higher stability standards depending on the other ingredients.

Surfactant concentration aids are typically selected from the group consisting of single long chain alkyl cationic surfactants; nonionic surfactants; amine oxides; fatty acids; or mixtures thereof, typically used at a level of from 0 to about 15% of the composition.

Such mono-long-chain-alkyl cationic surfactants useful in the present invention are, preferably, quaternary ammonium salts of the general formula:



wherein the  $R^2$  group is  $C_{10}$ – $C_{22}$  hydrocarbon group, preferably  $C_{12}$ – $C_{18}$  alkyl group of the corresponding ester linkage interrupted group with a short alkylene ( $C_1$ – $C_4$ ) group between the ester linkage and the N, and having a similar hydrocarbon group, e.g., a fatty acid ester of choline, preferably  $C_{12}$ – $C_{14}$  (coca) choline ester and/or  $C_{16}$ – $C_{18}$  tallow choline ester at from about 0.1% to about 20% by weight of the softener active. Each R is a  $C_1$ – $C_4$  alkyl or substituted (e.g., hydroxy) alkyl, or hydrogen, preferably methyl, and the counterion  $X^-$  is a softener compatible anion, for example, chloride, bromide, methyl sulfate, etc.

Other cationic materials with ring structures such as alkyl imidazoline, imidazolinium, pyridine, and pyridinium salts having a single  $C_{12}$ – $C_{30}$  alkyl chain can also be used. Very low pH is required to stabilize, e.g., imidazoline ring structures.

Some alkyl imidazolinium salts and their imidazoline precursors useful in the present invention have the general formula:



wherein  $\text{Y}^2$  is  $-\text{C}(\text{O})-\text{O}-$ ,  $-\text{O}-(\text{O})\text{C}-$ ,  $-\text{C}(\text{O})-\text{N}(\text{R}^5)-$ , or  $-\text{N}(\text{R}^5)-\text{C}(\text{O})-$  in which  $\text{R}^5$  is hydrogen or a  $C_1$ – $C_4$  alkyl radical;  $\text{R}^6$  is a  $C_1$ – $C_4$  alkyl radical or H (for imidazoline precursors);  $\text{R}^7$  and  $\text{R}^8$  are each independently selected from R and  $R^2$  as defined hereinbefore for the single-long-chain cationic surfactant with only one being  $R^2$ .

Some alkyl pyridinium salts useful in the present invention have the general formula:

5



wherein  $R^2$  and  $X^-$  are as defined above. A typical material of this type is cetyl pyridinium chloride.

#### Nonionic Surfactant (Alkoxylated Materials)

Suitable nonionic surfactants for use herein include addition products of ethylene oxide and, optionally, propylene oxide, with fatty alcohols, fatty acids, fatty amines, etc.

Suitable compounds are substantially water-soluble surfactants of the general formula:



wherein  $R^2$  is selected from the group consisting of primary, secondary and branched chain alkyl and/or acyl hydrocarbyl groups; primary, secondary and branched chain alkenyl hydrocarbyl groups; and primary, secondary and branched chain alkyl- and alkenyl-substituted phenolic hydrocarbyl groups; said hydrocarbyl groups having a hydrocarbyl chain length of from 8 to 20, preferably from 10 to 18 carbon atoms. Y is typically  $-\text{O}-$ ,  $-\text{C}(\text{O})\text{O}-$ ,  $-\text{C}(\text{O})\text{N}(\text{R})-$ , or  $-\text{C}(\text{O})\text{N}(\text{R})\text{R}-$ , in which  $R^2$  and R, when present, have the meanings given hereinbefore, and/or R can be hydrogen, and z is at least 8, preferably at least 10–11.

The nonionic surfactants herein are characterized by an HLB (hydrophilic-lipophilic balance) of from 7 to 20, preferably from 8 to 15.

Examples of particularly suitable nonionic surfactants include

Straight-Chain, Primary Alcohol Alkoxylates such as tallow alcohol-EO(11), tallow alcohol-EO(18), and tallow alcohol-EO(25);

Straight-Chain, Secondary Alcohol Alkoxylates such as 2- $C_{16}$ EO(11); 2- $C_{20}$ EO(11); and 2- $C_{16}$ EO(14);

Alkyl Phenol Alkoxylates, such as p-tridecylphenol EO(11) and p-pentadecylphenol EO(18), as well as

Olefinic Alkoxylates, and Branched Chain Alkoxylates such as branched chain primary and secondary alcohols which are available from the well-known "OXO" process.

#### Amine Oxides

Suitable amine oxides include those with one alkyl or hydroxyalkyl moiety of 8 to 28 carbon atoms, preferably from 8 to 16 carbon atoms, and two alkyl moieties selected from the group consisting of alkyl groups and hydroxyalkyl groups with 1 to 3 carbon atoms.

Examples include dimethyloctylamine oxide, diethyldecyldamine oxide, bis-(2-hydroxyethyl)dodecylamine oxide, dimethyldodecyl-amine oxide, dipropyltetradecylamine oxide, methylethylhexadecylamine oxide, dimethyl-2-hydroxyoctadecylamine oxide, and coconut fatty alkyl dimethylamine oxide.

#### Fatty Acids

Suitable fatty acids include those containing from 12 to 25, preferably from 16 to 20 total carbon atoms, with the fatty moiety containing from 10 to 22, preferably from 10 to 14 (mid cut), carbon atoms. The shorter moiety contains from 1 to 4, preferably from 1 to 2 carbon atoms.

#### Electrolyte Concentration Aids

Inorganic viscosity control agents which can also act like or augment the effect of the surfactant concentration aids, include water-soluble, ionizable salts which can also option-

55

65

ally be incorporated into the compositions of the present invention. A wide variety of ionizable salts can be used. Examples of suitable salts are the halides of the Group IA and IIA metals of the Periodic Table of the Elements, e.g., calcium chloride, magnesium chloride, sodium chloride, potassium bromide, and lithium chloride. The ionizable salts are particularly useful during the process of mixing the ingredients to make the compositions herein, and later to obtain the desired viscosity. The amount of ionizable salts used depends on the amount of active ingredients used in the compositions and can be adjusted according to the desires of the formulator. Typical levels of salts used to control the composition viscosity are from about 20 to about 20,000 parts per million (ppm), preferably from about 20 to about 11,000 ppm, by weight of the composition.

Alkylene polyammonium salts can be incorporated into the composition to give viscosity control in addition to or in place of the water-soluble, ionizable salts above. In addition, these agents can act as scavengers, forming ion pairs with anionic detergent carried over from the main wash, in the rinse, and on the fabrics, and may improve softness performance. These agents may stabilize the viscosity over a broader range of temperature, especially at low temperatures, compared to the inorganic electrolytes.

Specific examples of alkylene polyammonium salts include 1-lysine monohydrochloride and 1,5-diammonium 2-methyl pentane dihydrochloride.

Another optional ingredient is a liquid carrier. The liquid carrier employed in the instant compositions is preferably at least primarily water due to its low cost relative availability, safety, and environmental compatibility. The level of water in the liquid carrier is preferably at least about 50%, most preferably at least about 60%, by weight of the carrier. Mixtures of water and low molecular weight, e.g., <about 200, organic solvent, e.g., lower alcohol such as ethanol, propanol, isopropanol or butanol are useful as the carrier liquid. Low molecular weight alcohols include monohydric, dihydric (glycol, etc.) trihydric (glycerol, etc.), and higher polyhydric (polyols) alcohols.

Still other optional ingredients are stabilizers, such as well known antioxidants and reductive agents, Soil Release Polymers, bacteriocides, colorants, perfumes, preservatives, optical brighteners, anti ionisation agents, antifoam agents, enzymes and the like.

The invention will be further illustrated by means of the following examples.

### EXAMPLES

General molecular structures: C-(A)x-(B)y-(A)z-D

A. Effect of a water-soluble non-block copolymer (PVP) on the viscosity of block copolymer-stabilized lamellar droplet dispersions:

#### Polymer used:

| Polymer | C and D                      | A      | B   | x  | y | z  |
|---------|------------------------------|--------|-----|----|---|----|
| P-1     | methyl                       | ethoxy | PPT | 45 | 5 | 45 |
| P-2     | Poly vinyl pyrrolidone (PVP) |        |     |    |   |    |

#### Storage viscosities:

| Content/% of |      | 7 day storage viscosity at: |        |      |     |      |
|--------------|------|-----------------------------|--------|------|-----|------|
| P-1          | P-2  | 4                           | 10     | RT   | 35  | 50   |
| 0.33         | —    | S                           | >20000 | 1210 | 570 | 1730 |
| —            | 0.33 | S                           | S      | S    | 720 | 1230 |
| 0.33         | 0.33 | S                           | 6800   | 328  | 155 | 320  |
| 0.33         | 1.0  | S                           | 4500   | 700  | 323 | 530  |
| 0.33*        | 1.0* | S                           | 19300  | 560  | 435 | 1670 |

-continued

|      |     |   |        |     |     |     |
|------|-----|---|--------|-----|-----|-----|
| 0.66 | 1.0 | S | >20000 | 413 | 225 | 303 |
| 1.0  | 1.0 | S | 15200  | 385 | 200 | 230 |

5 \*Means that both polymers have been added to the water seat. Otherwise the polymers have been added after the perfume when still hot.

The viscosity has been measured using a Brookfield Viscometer. The method used is the standard method known by 10 persons skilled in the art.

B. Effect of hydrophilic and hydrophobic block lengths of EO/PO/EO triblock copolymers on the viscosity of lamellar droplet dispersions:

15 A is an ethoxy unit (EQ) and B is a relatively hydrophobic unit like propoxy (PO) or propylene terephthalate (PPT). C and D, as well as x and z, are the same. They are all hydroxyl groups, except for the reference polymer which has methyl end groups.

| 25                | Polymer        | # EO's | # PO's | F**   | Cps after storage:        |                            |  |
|-------------------|----------------|--------|--------|-------|---------------------------|----------------------------|--|
|                   |                |        |        |       | 3 days at RT <sup>1</sup> | 10 days at RT <sup>2</sup> |  |
| Reference         |                | 80     | 5**    | 1425  | S                         | 470                        |  |
| Synperonic L35    |                | 22     | 16     | 608   | S                         | —                          |  |
| Synperonic F38    |                | 88     | 16     | 1664  | S                         | —                          |  |
|                   |                | 6200   |        |       |                           |                            |  |
| 30                | Synperonic F87 | 120    | 39     | 6201  | 115                       | —                          |  |
| Synperonic F88    |                | 206    | 39     | 9555  | 180                       | —                          |  |
| Synperonic F108   |                | 297    | 56     | 19768 | 180                       | —                          |  |
| Pluronic PE 10400 |                | 50     | 56     | 5936  | 50                        | 73                         |  |
| Pluronic PE 10500 |                | 74     | 56     | 7280  | 333                       | 83                         |  |

\*The numbers 1 and 2 stand for the reduced and the full matrix, respectively. The difference between the two is that in the reduced matrix some of the emulsifiers/dispersants have been omitted.

\*\*PPT units, length equivalent to 15PO units.

C. Effect of the center block chemistry on the viscosity of 40 lamellar droplet dispersions:

C and D are end groups, A is an ethoxy unit and B is a relatively hydrophobic unit like propoxy (PO), propylene terephthalate (PPT), n-butoxy (BuO), hexadecylene (C16), or dodecylene (C12).

C and D, as well as x and z, are the same.

| 50  | Center   | Viscosity (cps) after 7 days storage: |    |    |        |     |    |    |    |
|-----|----------|---------------------------------------|----|----|--------|-----|----|----|----|
|     |          | block                                 | C  | x  | y      | 4   | 10 | RT | 35 |
| PPT | methyl   |                                       | 45 | 5  | 630    | 120 | 35 | 35 | 60 |
| PO  | methyl   |                                       | 55 | 17 | >20000 | 360 | 45 | 45 | 72 |
| PO  | methyl   |                                       | 63 | 13 | >20000 | 290 | 40 | 43 | 68 |
| PO  | hydroxyl |                                       | 40 | 16 | >20000 | 342 | 35 | 35 | 43 |
| BuO | methyl   |                                       | 43 | 9  | 1780   | 160 | 35 | 40 | 60 |
| BuO | methyl   |                                       | 50 | 14 | 7700   | 265 | 36 | 38 | 58 |
| C16 | methyl   |                                       | 75 | 1  | 1260   | 223 | 38 | 40 | 45 |
| C12 | methyl   |                                       | 60 | 1  | 1146   | 238 | 52 | 50 | 54 |

D. Effect of end-groups on the viscosity of lamellar droplet dispersions:

C and D are end groups, A is an ethoxy unit and B is a relatively hydrophobic unit like propoxy (PO) or propylene terephthalate (PPT).

C and D, as well as x and z, are the same.

| End group      | functionallity | B  | x  | y | Viscosity (cps) after 7 days storage: |        |      |        | 5  |
|----------------|----------------|----|----|---|---------------------------------------|--------|------|--------|----|
|                |                |    |    |   | 10                                    | RT     | 35   | 50° C. |    |
| Methyl         | PPT            | 40 | 5  |   | >20000                                | 128    | 40   | 85     |    |
| Hydroxyl       | PO             | 40 | 15 |   | S                                     | >20000 | 43   | 80     |    |
| Methyl         | PO             | 55 | 17 |   | 360                                   | 45     | 45   | 72     |    |
| Methyl         | PO             | 63 | 13 |   | 290                                   | 40     | 43   | 68     |    |
| Hydroxyl       | PO             | 40 | 16 |   | 342                                   | 35     | 35   | 43     | 10 |
| Acetate        | PO             | 40 | 15 |   | S                                     | 7800   | 98   | 193    |    |
| Trimethyl-     | PO             | 40 | 16 |   | 328                                   | 43     | 40   | 43     |    |
| amido chloride |                |    |    |   |                                       |        |      |        |    |
| Hydroxyl       | PO             | 14 | 30 |   | S                                     | S      | 4600 | 14400  |    |
| Methyl         | PO             | 14 | 30 |   | S                                     | S      | 5600 | 9400   |    |

S = solid, RT = room temperature/° C.

E. Effect of a block copolymer according to the invention on the viscosity stability as measured after 7 days storage.

Two experiments have been performed in different softener matrices.

|                     | 4° C. | 10° C. | RT | 35° C. | 50 ° C. |    |
|---------------------|-------|--------|----|--------|---------|----|
| 1. w/o polymer P-1* | S     | S      | S  | S      | S       |    |
| with 0.5% P-1       | S     | S      | 88 | 160    | 235     |    |
| 2. w/o polymer P-1  | 360   | 123    | 78 | 113    | 235     | 25 |
| with 0.5% P-1       | 40    | 40     | 40 | 68     | 153     |    |

\*for P-1 description see Table A.

A typical formulation in above-mentioned examples for use as a rinse conditioner to which the different polymers were added, according to the invention comprises

|                 | weight % |  |
|-----------------|----------|--|
| Softener active | 24.5     |  |
| PGMS            | 2.0      |  |
| TEA 25          | 1.5      |  |
| HCl             | 0.12     |  |
| Antifoam agent  | 0.019    |  |
| Blue dye        | 80 ppm   |  |
| CaCl2           | 0.35     |  |
| Perfume         | 0.90     |  |

In conclusion above results clearly show:

- Beyond a certain length of the ethoxy side blocks the triblock copolymers provide a reduction of the product viscosity.
- The more hydrophobic the center block becomes the better the polymer stabilizes the viscosity.
- The combination of PVP with a triblock copolymer such as H3C-(EO)45-(PT)5-(EO)45-CH3 provides the best

viscosity stabilizing benefits. This MAY be due to PVP providing a shield around the positive charges such that the center block of the polymer adheres even better to the droplets.

What is claimed is:

- A liquid fabric softening composition comprising
  - from 0.1–10% of block copolymer with a hydrophobic backbone and one or more hydrophilic side chains, said block polymer being selected from the groups consisting of polymers having the formula:
    - C-(A)x-(B)y-D wherein A are water-soluble monomers and B are insoluble or partially water-soluble monomers, C and D are end-groups or a hydrogen atom; x and y are integers from 1–200,
    - C-(A)x-(B)y-(A)z-D wherein A are water-soluble monomers and B are insoluble or partially water-soluble monomers; C and D are end-groups or a hydrogen atom; x, y and z are integers from 1–200,
    - D-(A)x-R-(A)z-C wherein R is an insoluble or partially water-soluble monomer or a fatty alcohol or acid of which one carbon is substituted with polymer blocks, A are water-soluble monomers, C and D are end groups or a hydrogen atom, x and y are integers of from 1–200; and
  - from 0.1 to 10% of a non-ionic water-soluble polymer selected from the group consisting of polyvinylpyrrolidone, polyvinylpyridine-N-oxide, polyethylene glycol and substituted polyglycols; and
  - from 1% to 80% of fabric softener active.
- A fabric softening composition according to claim 1 wherein components a and b are in a ratio of a/b which ranges from 0.01 to 100.
- A fabric softening composition according to claim 1 wherein the integers x and z range from 30–60 and y ranges from 3–50.
- A fabric softening composition according to claim 3 wherein the integers x and z range from 30–60 and y ranges from 40–50.
- The composition of claim 4 wherein component c) is a quaternary ammonium fabric softener.
- The composition of claim 5 wherein the amount of component c) is from 5% to 50%.
- The composition of claim 6 wherein the amount of component a) is from 0.2 to 6% and the amount of component b) is from 0.2 to 6%.
- The composition of claim 7 wherein the amount of component c) is from 15% to 35%.

\* \* \* \* \*